



US007749565B2

(12) **United States Patent**  
**Johnson et al.**

(10) **Patent No.:** **US 7,749,565 B2**  
(45) **Date of Patent:** **Jul. 6, 2010**

(54) **METHOD FOR APPLYING AND  
DIMENSIONING AN ABRADABLE COATING**

(75) Inventors: **Curtis Alan Johnson**, Niskayuna, NY (US); **Yuk-Chiu Lau**, Ballston Lake, NY (US); **Joshua Lee Margolies**, Niskayuna, NY (US); **Herbert Chidsey Roberts, III**, Simpsonville, SC (US)

(73) Assignee: **General Electric Company**, Schenectady, NY (US)

(\*) Notice: Subject to any disclaimer, the term of this patent is extended or adjusted under 35 U.S.C. 154(b) by 767 days.

(21) Appl. No.: **11/537,278**

(22) Filed: **Sep. 29, 2006**

(65) **Prior Publication Data**

US 2010/0124608 A1 May 20, 2010

(51) **Int. Cl.**

**B05D 3/00** (2006.01)

(52) **U.S. Cl.** ..... **427/271**; 427/448; 427/154; 427/356; 427/357

(58) **Field of Classification Search** ..... **427/271**, 427/448, 154, 356, 357

See application file for complete search history.

(56)

**References Cited**

**U.S. PATENT DOCUMENTS**

|                 |        |                    |         |
|-----------------|--------|--------------------|---------|
| 6,503,574 B1 *  | 1/2003 | Skelly et al. .... | 427/446 |
| 6,887,528 B2    | 5/2005 | Lau et al.         |         |
| 2004/0005452 A1 | 1/2004 | Dorfman et al.     |         |
| 2005/0003172 A1 | 1/2005 | Wheeler et al.     |         |
| 2006/0110247 A1 | 5/2006 | Nelson et al.      |         |
| 2006/0110248 A1 | 5/2006 | Nelson et al.      |         |

**FOREIGN PATENT DOCUMENTS**

|    |             |         |
|----|-------------|---------|
| EP | 1548144 A1  | 11/2004 |
| WO | 02099254 A1 | 12/2002 |
| WO | 03026886 A2 | 4/2003  |

**OTHER PUBLICATIONS**

EP Search Report for Application No. 07117320.7, dated Mar. 5, 2009.

\* cited by examiner

*Primary Examiner*—Roberts Culbert

(74) *Attorney, Agent, or Firm*—Cantor Colburn LLP

(57) **ABSTRACT**

Disclosed is a coated substrate including a substrate coating applied to at least one substantially flat surface of the substrate, the coating including at least one of an axial concavity and a circumferential curvature, the substrate being configured for disposal parametrically about a moving component.

**9 Claims, 10 Drawing Sheets**



FIG. 1



FIG. 2



FIG. 3



FIG. 4



FIG. 5



FIG. 6



FIG. 7



FIG. 8



FIG. 9



**FIG. 10**

## 1

METHOD FOR APPLYING AND  
DIMENSIONING AN ABRADABLE COATING

## FIELD OF THE INVENTION

The disclosure relates generally to a method for applying an abradable coating to a substrate, and more specifically to a method for applying and dimensioning the abradable coating.

## BACKGROUND OF THE INVENTION

In a gas turbine engine, in order to achieve maximum engine efficiency (and corresponding maximum electrical power generation), it is important that the buckets rotate within the turbine casing or "shroud" with minimal interference and with the highest possible efficiency relative to the amount of energy available from the expanding working fluid. Typically, highest operation efficiencies can be achieved by maintaining a minimum threshold clearance between the shroud and tips of the bucket. Maintaining a minimum clearance prevents unwanted "leakage" of a hot gas over tip of the buckets, increased clearances lead to leakage problems and cause significant decreases in overall efficiency of the turbine. However, it should be appreciated that if bucket tips rub against a particular location of the shroud such that the bucket tip is eroded, the erosion of the bucket tip increases clearances between bucket tip and shroud in other locations, again resulting in unwanted leakage.

The need to maintain adequate clearance without significant loss of efficiency is made more difficult by the fact that as the turbine rotates, centrifugal forces acting on the turbine components can cause the buckets to expand in an outward direction toward the shroud, particularly when influenced by the high operating temperatures. Thus, it is important to establish the lowest effective running clearances between the shroud and bucket tips at the maximum anticipated operating temperatures.

Abradable type coatings have been applied to the turbine shroud to help establish a minimum, i.e., optimum, running clearance between the shroud and bucket tips under steady-state temperature conditions. In particular, coatings have been applied to the surface of the shroud facing the buckets using a material that can be readily abraded by the tips of the buckets as they turn inside the shroud at high speed with little or no damage to the bucket tips. Initially, a clearance exists between the bucket tips and the coating when the gas turbine is stopped and the components are at ambient temperature. Later, during normal operation the clearance decreases due to the centrifugal forces and temperature changes in rotating and stationary components inevitably resulting in at least some radial extension of the bucket tips, causing them to contact the coating on the shroud and wear away a part of the coating to establish the minimum running clearance. With abradable coatings clearances can be reduced with the assurance that if contact occurs, the sacrificial part is the abradable coating instead of the bucket tip.

Typically, the shrouds to which abradable coatings are applied to are fabricated (i.e. machined or cast) to include a concave profile that mates with a convex contour of a surface of the bucket tips (the rotation of the bucket tip will form a convex contour towards the shroud, though it should be appreciated that the surface of each bucket tip is not necessarily convex, and may be flat). Mating the concavely machined shroud with the convex bucket tip in this manner maintains a minimum clearance over the whole surface of the tip. Since an abradable coating applied to a concavely machined shroud includes the profile of the shroud to which

## 2

it is applied, the abradable coating is also concavely disposed to mate with the convex tip. However, manufacturing a shroud to include the concave profile, or any desired profile, can be difficult and expensive. Thus, a method that would allow the abradable coating to include a profile that matches the profile of the bucket tips with which it interacts without machining the shroud is desirable.

## BRIEF DESCRIPTION OF THE INVENTION

Disclosed is a coated substrate including a substrate coating applied to at least one substantially flat surface of the substrate, the coating including at least one of an axial concavity and a circumferential curvature, the substrate being configured for disposal parametrically about a moving component.

Also disclosed is a method for applying and dimensioning a substrate coating, the method including applying at least one substrate layer to at least one surface of a substrate, creating the substrate coating via the applying of the at least one substrate layer, intentionally removing a portion of coating material from the at least one substrate layer via at least one moving component operating in proximity to the substrate, and shaping the substrate coating to include a desired profile via the removing.

Further disclosed is a method for applying and dimensioning a substrate coating, the method including applying at least one substrate layer to at least one flat surface of a substrate, the substrate being configured for disposal parametrically about a moving component, creating the substrate coating via the applying of the at least one substrate layer, and shaping at least one of the at least one substrate layers to include at least one of an axial concavity and a circumferential curvature.

## BRIEF DESCRIPTION OF THE DRAWINGS

Referring now to the drawings wherein like elements are numbered alike in the several FIGURES:

FIG. 1 is a schematic cross-section of a side view of an abradable coating applied to a substrate including a substantially flat surface.

FIG. 2 is a schematic cross-section of side view of the abradable coating applied to a substrate including a substantially flat surface and a moving component operating in proximity to the substrate;

FIG. 3 is a schematic cross-section of a side view of the abradable coating applied to a substrate including a substantially flat surface, wherein the coating has been shaped;

FIG. 4 is a schematic representation of a side view of the abradable coating applied to a substrate including a substantially flat surface;

FIG. 5 is a schematic representation of a side view of the abradable coating applied to a substrate including a substantially flat surface and a moving component operating in proximity to the substrate;

FIG. 6 is a schematic representation of a side view of the abradable coating applied to a substrate including a substantially flat surface, wherein the coating has been shaped;

FIG. 7 is a schematic cross-section of a side view of the abradable coating applied to a substrate in accordance with an alternate embodiment, wherein the substrate includes a substantially flat surface and the coating has been shaped;

FIG. 8 is a schematic representation of a side view of the abradable coating applied to a substrate in accordance with an alternate embodiment, wherein the substrate includes a substantially flat surface and the coating has been shaped;

FIG. 9 is a block diagram illustrating a method for applying and dimensioning the abradable coating;

FIG. 10 is a block diagram illustrating a method for applying and dimensioning the abradable coating.

As is known in the art, maintaining a minimum threshold clearance 21 between the shroud 12 and the tip 22 of the bucket 24 is desirable. Because of this desire to maintain threshold clearance 21 at a minimum, the tip 22 of the bucket 24 can sometimes come into contact with at least one of the layers 16 and 18 of the coating 10. Because, in an exemplary embodiment, the bucket tip 22 is convex towards the flat surface 14 (it should be appreciated that the tip 22 may also be flat), contact between the bucket tip 22 and flat coating 10 10 occurs most frequently at an extended relative centerline 26 of the shroud 12, where the threshold clearance 21 is at its least. As the threshold clearance 21 becomes larger away from the centerline 26 (in a direction of either side 28 of the shroud 12), contact between the bucket tip 22 and the flat 15 coating 10 occurs less frequently. As such, less material is removed from the coating 10 in regions of the coating successively further from the centerline 26, creating a concave profile in the coating 10 in relation to the tip 22, as shown in FIGS. 2 and 3. Thus, the convex rotating tip 22 may be used 20 to intentionally shape the desired axial concavity 30 in the coating. In addition, it should be appreciated that a rotating tip 22 (or moving component of any kind that operates in proximity the shroud or substrate) may be chosen to include a desirable shape (concave, convex, or otherwise) that will 25 move/rotate to shape an abradable coating via a removal of abradable material caused by the moving/rotating.

Additionally, a portion of abradable material of at least one of the abradable layers 16 and 18 may be removed, via the moving component 22, to create a circumferential curvature 30 30 41 in the shroud 12, as shown in FIGS. 4-6. As in the exemplary embodiment above, the moving component 22 may be a tip of a bucket that is associated with the rotor 23 and rotating during operation of a turbomachine (not illustrated in its entirety). Again, though the moving component 22 will not be limited to a blade tip, for purposes of clarity and simplicity the moving component 22 will be referred to as the tip 22 of the rotating bucket 24 hereinafter.

Referring to FIG. 4, the shroud 12 may include a plurality of shroud segments 44 (the shroud 12 may include any number of segments 44, with an exemplary embodiment including 96 or 120). Each segment 44 is shown with the coating 10 having been applied to its substantially flat surface 14, wherein the originally applied coating 10 also includes a substantially flat coating surface 45. As mentioned above, the tips 22 of the bucket 24 can sometimes come into contact with the coating 10, as shown in FIG. 5. As the bucket tips 22 rotate during operation of the machine, contact between the bucket tips 22 and flat coating 10 occurs most frequently at a relative center region 42 of each shroud segment 44 of the shroud 12. 45 This leads to abradable material removal (particularly from, though not limited to the patterned layer 18) most prominently at the center region 42 of the shroud segments 44, where a radial distance from the rotor 23 is at a minimum relative to edges 46 of the shroud segments 44. This removal 50 creates the circumferential curvature 41, such as that illustrated in FIG. 6. Thus, the rotating tip 22 may be used to intentionally shape the desired circumferential curvature 41 and axial concavity 30 in the coating 10. In addition, it should be appreciated that a rotating tip 22 (or moving component of any kind that operates in proximity to the shroud or substrate) may be chosen to include a desirable shape (concave, convex, or otherwise) that will move/rotate to shape an abradable coating, as desirable, via a removal of abradable material caused by the moving/rotating.

65 Furthermore, it should be appreciated that the layers 16 and 18, particularly the patterned layer 18, may be applied in such a manner that a sufficient portion (at least about 50% of an

## DETAILED DESCRIPTION

Referring to FIG. 1, a substrate coating, such as an abradable coating 10, is shown applied to a substrate 12 including a substantially flat surface 14, wherein the coating 10 is applied in at least one substrate layer, such as abradable layers 16 and 18. In an exemplary embodiment, the substrate 12 is a turbine shroud, to which the coating 10 is applied in an adhering layer and a patterned layer. Though the substrate 12 will not be limited to a turbine shroud, and the at least one layer 16 and 18 will not be limited to an adhering layer and a patterned layer, for purposes of clarity and simplicity, the substrate 12 will be referred to as the shroud 12, and the at least one layer 16 and 18 will be referred to as the adhering layer 16 and the patterned layer 18 hereinafter.

The adhering layer 16 is applied to the substantially flat surface 14 of the shroud 12, which will typically be environmental barrier coated (EBC). The adhering layer 16 may be a metallic bond coat, such as MCrAlY, or a ceramic layer such as yttria stabilized zirconia or barium strontium aluminosilicate. The layer 16 may be applied via a powder that is cut to any desired size or coarseness, and then sprayed or flash coated, though application is not limited to these methods, onto the shroud 12 via a thermal spray process, such as air plasma spray or physical vapor deposition (PVD).

Applied to the adhering layer 16 is the patterned layer 18. The patterned layer 18 will typically be a ceramic layer, such as yttria stabilized zirconia or barium strontium aluminosilicate. The layer 18 may be applied via a powder that is cut to any desired size or coarseness, and then sprayed onto the adhering layer 16 through a patterned mask disposed on the adhering layer 16, though application is not limited to inclusion of the patterned mask. In an exemplary embodiment, the powder that will be the patterned layer 18 may be applied via a thermal spray process, such as air plasma spray, wherein the powder may be applied in multiple passes of air plasma spray. Alternatively, a PVD coating would be built up with prolonged exposure to the vapor phase of the coating material after it had similarly passed through a patterned mask. The patterned layer 18 left behind by the patterned mask defines at least one ridge 20. It should be appreciated that application of the coating 10 may also include a heat treatment of the layers 16 and 18 (though application is not limited to inclusion of this treatment), which may aid in bonding and strengthening of the layers (to help avoid coating erosion), and creating a desired coating porosity. By applying the layer 16 and 18 as discussed hereinabove, the abradable coating 10 is created on the shroud 12, and includes the shrouds essentially flat profile.

With the coating 10 having been created on the shroud 12, a portion of abradable material of at least one of the abradable layers 16 and 18 may be removed, creating an axial concavity 30 in the shroud, via a moving component 22, as shown in FIG. 2 and. In an exemplary embodiment, the moving component 22 may be a tip of a bucket that is associated with a rotor 23 (see FIGS. 5-6) and rotating during operation of a turbomachine (not illustrated in its entirety). Though the moving component 22 will not be limited to a blade tip, for purposes of clarity and simplicity the moving component 22 will be referred to as the tip 22 of the rotating bucket 24 hereinafter.

original ridge height **40** in an exemplary embodiment) of the layer **18** will remain following intentional shaping via the rotating tip **22**. For example, as shown in an exemplary embodiment illustrated in FIGS. 2 and 3, the ridges **20** of the layer **18** may be created to include an original height **32** that is sized to prevent more than about 50% of any of the ridges **21** from being abraded by the rotating tip **22**. Sizing the ridges **21** in this manner makes it likely that at least a portion of the abradable layers **16** and **18** will remain intact after shaping, and that some of this portion will continue to include any aerodynamic benefits of the at least partially remaining ridges **21**. It should be appreciated however, that some regions of the layer **18** may have more than 50% of abradable material eroded away during shaping.

In addition, referring again to FIGS. 3 and 6, as well as 7 and 8, at least one of the layers **16** and **18** may also be either machined or applied in a selective manner to create a variable thickness (see relatively thicker regions **50a** and **50b**) in at least one of the layers **16** and **18**, to create at least one of the desired axial concavity **30** or a circumferential curvature **41**. For example, in FIGS. 3 and 6 the patterned layer **18** may have been applied to the adhering layer **16**, with the patterned layer **18** (or both layers **16** and **18**) either having been applied more thickly at the selected thicker regions **50a** and **50b**, or applied evenly and then machined at the areas of the centerline **26** (for axial concavity **30**) and/or center region **42** (for circumferential curvature **41**) to create the desired profile. Referring to FIGS. 7 and 8, the adhering layer **16** may also be first applied to the shroud surface(s) **14**, either more thickly at the selected thicker regions **50a** and **50b**, or evenly across the surface **14**, with the layer **16** then being machined at the areas of the centerline **26** (for axial concavity **30**) and/or center region **42** (for circumferential curvature **41**) to create the desired profile. Whether one or both of the layers **16** and **18** is applied more thickly at selected regions, applied evenly and machined in a desired fashion, or applied evenly and intentionally removed via the blade tip **22**, the end result is a coating **10** that is applied to the flat surface **14**, but includes a desired axial concavity **30** and/or circumferential curvature **41**. Referring to the machining of the layers **16** and **18**, it should be appreciated that machining can be accomplished via any desired process, such as but not limited to grinding (in an exemplary embodiment), cutting, ultrasonic machining, and laser ablating.

It should still further be appreciated that the coating **10** referred to throughout the disclosure may be any type of abradable coating (such as a continuous porous metallic coating) including and applied in any number of coating layers.

Referring to FIG. 9, a method **100** for applying and dimensioning an abradable coating is illustrated in a block diagram. The method **100** includes applying at least one abradable layer **16/18** to a surface of a substrate, as shown in operational block **102**, wherein the substrate may be a turbine shroud **12** including a substantially flat surface **14**. The method **100** also includes creating the abradable coating **10** via the applying of the at least one abradable layer **16/18** and intentionally removing a portion of abradable material from the at least one abradable layer **16/18** via at least one moving component, such as a tip **22** of a rotating bucket **24**, operating in proximity to said substrate, as shown in operational block **104**. The method **100** further includes shaping the abradable coating **10** to include a desired profile, such as an axial concavity **30** and/or circumferential curvature **41**, via said removing, as shown in operational block **106**.

Referring to FIG. 10, a method **200** for applying and dimensioning a substrate coating **10** is illustrated and includes applying at least one substrate layer **16/18** to at least one flat surface **14** of a substrate **12**, the substrate **12** being configured for disposal parametrically about a moving com-

ponent **24**, as shown in operational block **202**. The method **200** also includes creating the substrate coating **10** via the applying of the at least one substrate layer **16/18**, and shaping at least one of the at least one substrate layers **16/18** to include at least one of an axial concavity **30** and a circumferential curvature **41**, as shown in operational block **204**.

While the invention has been described with reference to an exemplary embodiment, it should be understood by those skilled in the art that various changes may be made and equivalents may be substituted for elements thereof without departing from the scope of the invention. In addition, many modifications may be made to adapt a particular situation or substance to the teachings of the invention without departing from the scope thereof. Therefore, it is important that the invention not be limited to the particular embodiment disclosed as the best mode contemplated for carrying out this invention, but that the invention will include all embodiments falling within the scope of the apportioned claims. Moreover, unless specifically stated any use of the terms first, second, etc. do not denote any order or importance, but rather the terms first, second, etc. are used to distinguish one element from another.

What is claimed is:

1. A method for forming a substrate coating, the method comprising:

forming a shroud to perimetrically surround a moving component, which is rotatable about a longitudinal axis of the shroud;

applying a substrate layer to an interior surface of the shroud to form the substrate coating with a plurality of substantially flat interior facing surfaces each meeting an adjacent surface to form an obliquely angled edge; and

rotating the moving component within the shroud to selectively remove a portion of the substrate coating via contact between the substrate layer at each of the interior facing surfaces and the moving component to thereby shape each of the interior facing surfaces to respectively include:

an axial profile having an axial concavity complementary to a radial curvature of an axial shape of a tip of the moving component and a circumferential curvature complementary to a pattern traced by the tip of the moving component.

2. The method according to claim 1, wherein the substrate layer comprises an abradable coating.

3. The method according to claim 1, wherein the substrate layer comprises an adhering layer and a patterned layer.

4. The method according to claim 1, wherein the applying of the substrate layer comprises applying an adhering layer to the interior surface of the shroud.

5. The method according to claim 1, wherein the applying of the substrate layer comprises creating at least one ridge in the substrate layer.

6. The method according to claim 5, wherein the creating of the at least one ridge comprises creating the at least one ridge with an original height that will remain at least about 50 percent following the selective removal of the portion of the substrate.

7. The method according to claim 5, wherein the creating comprises machining of the substrate layer.

8. The method according to claim 1, wherein the applying of the substrate layer comprises allowing for the axial concavity and the circumferential curvature.

9. The method according to claim 1, wherein the moving component comprises a rotating turbine bucket.